

R. GAHL.

PROCESS OF RECOVERING METALS FROM ORES.

APPLICATION FILED NOV. 8, 1917.

1,291,824.

Patented Jan. 21, 1919.



Rudolf Gahl  
by  
Byers, Townsend & Nichols  
Inventor  
Attorneys.

# UNITED STATES PATENT OFFICE.

RUDOLF GAHL, OF MIAMI, ARIZONA.

## PROCESS OF RECOVERING METALS FROM ORES.

1,291,824.

Specification of Letters Patent. Patented Jan. 21, 1919.

Application filed November 8, 1917. Serial No. 200,931.

*To all whom it may concern:*

Be it known that I, RUDOLF GAHL, a citizen of the United States, residing at Miami, in the county of Gila and State of Arizona, have invented certain new and useful Improvements in Processes of Recovering Metals from Ores, of which the following is a specification.

My invention relates to a process of recovering metals from ores. For the beneficiation of certain ores, especially porphyry copper ores by means of concentration processes, very fine grinding is necessary to liberate the economic mineral from the gangue particles and from particles of such minerals as cannot be recovered by the concentration process. The cost of grinding, therefore, often constitutes the heaviest item of the reduction cost by the processes in question.

For this and other reasons, it has been customary to reduce the grinding expense by not attempting to carry the grinding as far as is necessary for freeing all mineral from gangue particles, but to apply the concentrating process to what may be called insufficiently crushed ore. The products which the concentration process yields in this case are so-called "concentrate" containing essentially those mineral particles that have been liberated largely from the gangue and a "middling" product containing particles consisting of gangue and mineral combined, in addition to a waste product called "tailing".

It has been customary in such cases to regrind the middling product and then to attempt another concentration.

While the procedure just described has been successful in a measure, it does not permit essentially complete recovery of the mineral contents of the ore in the form of a high-grade product. The two principal causes for this shortcoming are (1) a great number of insufficiently ground particles find their way into the tailing product instead of going into the middling product; and (2) the treatment of the reground middling product by a concentration process is rarely satisfactory, inasmuch as the resulting tailing always carries high mineral values. The reason seems to lie in the fact that altered or partly decomposed minerals

which offer difficulties in concentration processes accumulate to some extent in the middling product.

In speaking of concentration processes so far, I have been referring to gravity concentration processes only. As a matter of fact, the flotation process which has recently come into use is also a concentration process.

In applying the flotation process, metallurgists have generally confined themselves to applying the same to slimes, *i. e.*, very fine crushed portions of ore; or when they have applied it to ore pulps as a whole, *i. e.*, sand and slime mixed, have specified that the crushing should be very fine.

I have discovered, however, that the flotation process may be so carried out that it is well adapted to the treatment of insufficiently crushed ore, and that when so applied, in the manner hereinafter described, there will be produced, in contradistinction to the gravity process, a tailing product practically free from mineral values, while the flotation concentrates contain mineral particles essentially free from gangue and the middlings contain mineral particles combined with the gangue. The separation into these three products is not necessarily made in one operation. As in the example quoted below, the first flotation may, for instance, separate out the concentrate and an additional treatment of the balance of the pulp result in the middling and tailing product.

My experience is further, that flotation, like the gravity concentration process, does not permit the separation of the middling product into a mineral free secondary tailing product and a high-grade secondary concentrate product even after regrinding. On the other hand, I have discovered that the middling product can be obtained in a granular form suitable for roasting and leaching, if the flotation in which the middling is produced is applied to a pulp from which the slime has been previously removed by means known to the art, as for instance, a drag classifier. Such roasting treatment followed by leaching permits a high extraction of the values contained in the middlings product.

It has been mentioned before that the flotation process will produce a tailing product practically free from mineral

values in addition to a concentrate and a middling product refractory to further treatment by flotation. The term "practically free from mineral values" is meant to apply only to such mineral values as are amendable to flotation. Where, for instance, oxidized copper ores are treated, it is only possible to remove the copper sulfids with a very high degree of extraction, while the copper carbonates are extracted to a smaller extent, and silicates to a smaller extent yet. Where the oxid minerals exist in a sufficiently large percentage, another method may have to be used to supplement the flotation treatment, and I prefer leaching for this purpose.

As an example of my process, a copper ore was ground so that practically all the product was fine enough to pass a 48-mesh screen, which though comparatively fine grinding is by no means sufficient to liberate all the mineral particles. The ore treated contained approximately 1.5% copper, 0.3% being in oxid combination. As the result of a combined gravity and flotation concentration, a concentrate containing about 30% of copper was produced.

The tailings from this concentration process, which would ordinarily be considered waste product, were then, after the removal of the slime, separated into a middling and tailing product in a flotation machine. While the material fed to this flotation machine carried 0.26% copper, the tailing product contained only 0.11% copper, and after leaching with sulfuric acid contained only 0.04% copper.

The middling product, containing 1.70% copper was roasted with salt and then leached with sulfuric acid, and by this process the copper content of the residue was reduced to 0.09% copper. In other words, the loss originating from this waste product was also very small.

The copper solutions produced by leaching the tailings and by leaching the roasted middlings can then be treated either by precipitating the copper on iron to produce cement copper, or by electrolytic deposition.

The attached figure represents part of a

flow-sheet of a process, which, although deviating somewhat from the procedure just described, shows the application of the underlying principle. From this flow sheet, details like settling tanks, filters, feeders, 55 are omitted. As shown in this flow sheet, the ore is first crushed, the crushed ore then deslimed, and the sand passed to flotation machine No. 1, the concentrates from this machine being sent to flotation machine 60 No. 2, the tails from both machines being sent to flotation machine No. 3. The middlings produced by flotation in this machine are sent to a roasting furnace in which they are given a chloridizing roast, 65 and then together with the unroasted tailings sent to the leaching plant. From the resulting solutions, the copper is recovered either by precipitation as cement copper or as electrolytic copper, and the residues from 70 the leaching are discarded.

The slimed product from the desliming classifier may be treated in any of the well known ways.

I claim:

1. The process of treating ores which consists in subjecting deslimed pulp to flotation to produce a middling product, roasting the middling product, and leaching the roasted product to obtain a metalliferous 75 solution.

2. The process of treating ores which consists in subjecting deslimed pulp to flotation to produce a middling product, roasting the middling product, and leaching the 80 roasted product and the tailings to obtain a metalliferous solution.

3. The process of treating ores which consists in subjecting deslimed pulp to flotation to produce concentrates and tailings, 85 subjecting such tailings to flotation to produce a middling product, roasting the middling product, and leaching the roasted product to obtain a metalliferous solution.

4. The process as claimed in claim 3 including the step of also leaching the tailings from the flotation process in which the middling product was obtained.

In testimony whereof I affix my signature.  
RUDOLF GAHL.